

# UNITED STATES PATENT OFFICE.

FREDERICK M. BECKET, OF NIAGARA FALLS, NEW YORK, ASSIGNOR TO  
ELECTRO METALLURGICAL COMPANY, A CORPORATION OF WEST  
VIRGINIA.

## ALLOY AND METHOD OF PRODUCING IT.

No. 858,327.

Specification of Letters Patent.

Patented June 25, 1907.

Application filed March 20, 1907. Serial No. 363,481.

*To all whom it may concern:*

Be it known that I, FREDERICK M. BECKET, a subject of the King of Great Britain, residing at Niagara Falls, in the county of Niagara and State of New York, have invented 5 certain new and useful Improvements in Alloy and Methods of Producing It, of which the following is a specification.

This invention relates to the production of 10 an alloy particularly adapted for the treatment of iron or steel, and to the method by which it is produced. The alloy contains titanium and calcium, preferably but not necessarily associated with aluminium and 15 silicon, carbon being usually present in greater or less proportion in accordance with the method of manufacture employed. Iron is also usually present as a component of the alloy, derived from the ores employed in its 20 manufacture.

I may produce an alloy containing titanium and calcium by reduction by carbon in an electric furnace of a charge containing oxides or oxygen compounds of titanium and 25 calcium, usually with the addition of silica in proportion depending upon the percentage of silicon desired. The reduction of the mixed oxides yields a product of metallic character instead of the carbid which would 30 result from the reduction of either oxid alone. In addition to its value as an ingredient of the alloy for use in the treatment of iron or steel, silicon acts to a marked degree to diminish the percentage of carbon in the product; this is of advantage for the reason that 35 a product low in carbon can be added, if desired, in relatively large proportions to iron or steel without unduly increasing the proportion of carbon in the resulting metal.

When an alloy containing aluminium in 40 addition to titanium and calcium is desired, it is most conveniently produced by reduction in an electric furnace having an electrode or electrodes of carbon, of a charge 45 containing oxides of titanium and calcium, or of titanium, calcium and silicon, by means of metallic aluminium used in proportion to yield an aluminum-bearing alloy; or a mixture of the oxides of titanium, calcium and aluminium, or of titanium, calcium, aluminium and silicon, may be reduced by 50 carbon.

In any case the operation is preferably 55 rendered continuous in character by adding fresh portions of the charge from time to time, and tapping the molten alloy as desired.

Examples of the composition of alloys I have produced for the purpose indicated are shown by the following analyses:

|           |       |           |       |           |    |
|-----------|-------|-----------|-------|-----------|----|
| Titanium  | 50.67 | per cent. | 26.24 | per cent. | 60 |
| Calcium   | 8.32  | "         | 5.30  | "         |    |
| Aluminium | 22.70 | "         | 1.55  | "         |    |
| Iron      | 11.83 | "         | 50.98 | "         |    |
| Silicon   | 4.20  | "         | 11.78 | "         | 65 |
| Carbon    | 1.86  | "         | 3.69  | "         |    |
| Total     | 99.58 |           | 99.54 |           |    |

It will be understood that the proportions of the several components of the alloy, or the presence therein of aluminium or silicon, is determined by the composition of the charge smelted. The alloy is varied in composition according to the percentage of one or more of its constituents desired in the finished iron or 75 steel, and also according to the particular class of iron or steel to be treated.

The appearance of the alloy varies in accordance with its composition, mode and scale of production, rate of cooling, etc.; in 80 general it exists as a light gray or grayish product of metallic appearance but without pronounced luster or distinct crystalline structure, of moderate hardness. Particularly when a considerable proportion of calcium is present it is subject to slow decomposition in water or moist air. As compared with ferrotitanium the alloy possesses a relatively low melting point and is much more readily incorporated with molten iron or 90 steel and distributed therethrough.

The method of treating iron or steel by incorporating therewith the above described alloy is claimed in my copending application Serial No. 362,224, filed March 13, 1907. 95

I claim:

1. An alloy containing titanium and calcium.
2. An alloy containing titanium, calcium and aluminium. 100
3. An alloy containing titanium, calcium, aluminium, and silicon.
4. An alloy containing titanium, calcium, aluminium, silicon, and carbon.
5. An alloy containing titanium, calcium, aluminium, silicon, carbon, and iron. 105
6. The method of producing an alloy containing titanium and calcium, which consists in reducing a charge containing the oxides or oxygen compounds of titanium and calcium. 110
7. The method of producing an alloy con-

- taining titanium and calcium, which consists in reducing by carbon in an electric furnace a charge containing the oxids or oxygen compounds of titanium and calcium.
- 5 8. The method of producing an alloy containing titanium, calcium and silicon, which consists in reducing a charge containing the oxids or oxygen compounds of titanium, calcium and silicon.
- 10 9. The method of producing an alloy containing titanium, calcium and silicon, which consists in reducing by carbon in an electric furnace a charge containing the oxids or oxygen compounds of titanium, calcium and silicon.
- 15 10. The continuous method of producing an alloy containing titanium and calcium, which consists in reducing a charge containing the oxids or oxygen compounds of titanium and calcium, adding fresh portions of the charge, and withdrawing the products as desired.
- 20 11. The continuous method of producing an alloy containing titanium and calcium, which consists in reducing by carbon in an electric furnace a charge containing the oxids or oxygen compounds of titanium and calcium, adding fresh portions of the charge, and withdrawing the products as desired.
- 25 12. The continuous method of producing an alloy containing titanium and calcium, which consists in reducing by carbon in an electric furnace a charge containing the oxids or oxygen compounds of titanium, calcium and silicon, adding fresh portions of the charge and withdrawing the products as desired.
- 30 35

In testimony whereof, I affix my signature in presence of two witnesses.

FREDERICK M. BECKET.

Witnesses:

CHAS. F. RANSOM,  
R. H. WARREN.